

Dec. 30, 1941.

F. E. DRUMMOND

2,268,022

DRYING OIL COMPOSITION

Filed April 10, 1939

FIG. 1.



FIG. 2.



FIG. 3.



FIG. 4.



Inventor  
FOLSOM E. DRUMMOND,  
Tavelmin & Tavelmin  
Attorneys

## UNITED STATES PATENT OFFICE

2,268,022

## DRYING OIL COMPOSITION

Folsom E. Drummond, Dayton, Ohio, assignor, by  
mesne assignments, to New Wrinkle, Inc., Wil-  
mington, Del., a corporation of Delaware

Application April 10, 1939, Serial No. 266,959

5 Claims. (Cl. 106—264)

My invention relates to coating compositions and more particularly to compositions of the drying oil and wrinkle finish type. The invention, however, is applicable broadly in the compounding of varnishes, paints, enamels, printing inks and the like.

One object of this invention is to provide a conjugated double bond modified oil composition wherein the drying of a coating film comprising the modified oil vehicle is controlled by varying the constituents so as to produce either a wrinkle film or a smooth non-wrinkle film as desired.

Another object is to accelerate the polymerization and oxidation of paint oil compositions by the incorporation of certain amounts of unsaturated fatty acid glycerides having poly-conjugated double bond molecular structure.

Another object is to provide a coating composition of the character described comprising unsaturated fatty acid compounds of the poly-conjugated double bond type modified by the addition of metallic driers having improved drying properties.

Another object is to control the rapidity of drying of the coating film by varying the percentage amount of unsaturated organic compounds having conjugated double bonds introduced into the coating.

Still another object of this invention is to control the drying rate and wrinkling effect by varying the amount and type of poly-conjugated double bond glyceride compounds whereby the non-wrinkle oils may be made to dry to a wrinkle finish.

A further object is to provide a method of producing fast drying coating composition of the drying oil type without the necessity of introducing metallic driers.

Another object is to provide a method of treating drying and semi-drying oils so as to substantially enhance their drying properties.

A still further object is to provide a method of treating non-wrinkle oils so as to make them function as wrinkle oils. In this way the use of high priced blown China-wood and oiticica oils or wrinkle resins may be avoided.

In the drawing:

Figure 1 is a view in perspective illustrating a surface having applied thereto a coating composition of this invention which is dried to a plain smooth surface;

Figure 2 is a similar view showing a like coating presenting a wrinkle finish;

Figures 3 and 4 are enlarged fragmentary sectional views taken on the line 3—3 of Figure 1 and 4—4 of Figure 2, respectively.

Referring to the drawing in detail, 5 designates a panel or suitable base material provided with a coating film 6 of the rapid drying smooth surface type. A like base material having a wrinkle surface finish coating 7 is illustrated in Figures 2 and 4. The surface comprises irregular folds 8 which are formed in the skin portion of the coating film due to the rapid drying of the surface.

I have discovered that the drying of coating compositions can be controlled so as to produce either rapid drying, smooth surface compositions or films drying to a wrinkle finish by varying the amount of compounds present having conjugated double bond structure as illustrated by the general formula:  $(-\text{CH}=\text{CH}-)_x$ , where  $x$  represents 2 or more. Examples of compounds which comprise conjugated double bonds are unsaturated acids such as follows:



These unsaturated fatty acid compounds are constituents of many fats, especially drying and 40 semi-drying oils. In general the higher the number of conjugated double bonds

$(-\text{CH}=\text{CH}-)$

45 in the compound the more readily reactive it is. Similarly under the same conditions the greater the percentage amount of conjugated double bond compound in the coating film the shorter is the drying time.

In the formulation of rapid drying coating compositions of the drying oil type, according to my invention, utilization is made principally of the triglycerides of the fatty acids having poly-conjugated double bond molecular structure as heretofore mentioned.

Typical examples which illustrate the glycerides employed are:

(a) Triglyceryl-isolinoleate



(b) Triglyceryl-isolinolenate



(c) Triglyceryl-elaeostearate



(d) Triglyceryl-licanate



(e) Triglyceryl-octadecatetraenate



By incorporating various amounts of the tri-unsaturated glycerides in the conventional non-wrinkling paint oils the drying properties may be greatly enhanced and the waterproofing and flexibility of the product increased. Further by compounding the paint oils with a sufficient amount of fatty acid triglyceride compounds having three or more conjugated double bonds in the molecular structure drying oils, such as linseed, perilla, soya bean and the like, paint oils may be made to function as a wrinkling oil similar to China-wood oil. For bringing this about the oil and glyceride are combined by heating so that the product contains sufficient amount of glyceride having 3 or more conjugated double bond linkage so that the desired drying properties can be obtained. The percentage by weight of the glyceride added varies with each oil but may comprise upwards of 50 per cent by weight for producing wrinkling drying oil products. In this case the percentage amount of triglyceride is preferably in the neighborhood of 90 per cent of the paint oil composition.

Preferably the triglycerides are used since they produce the most pronounced drying effect. However, the use of di-unsaturated glycerides in place of the tri or mixtures thereof may be employed if desired. Further utilization may be made of the fatty acids alone when a sufficient amount of glycerol or glyceride constituents is present in the oil mixture. The fatty acids alone in the absence of glycerol or glyceride compound do not exhibit good drying properties.

Formulations made using the glycerides having only 2 conjugated double bonds produce a drying oil paint vehicle having superior drying and waterproofing qualities to those of linseed oil. Addition of suitable metallic driers to these modified drying oil vehicles will further enhance the drying of the composition to a smooth-non-wrinkling film when applied and air dried or baked at low temperatures.

Typical examples of non-wrinkling oil vehicles are as follows:

Example 1

|                            | Per cent by weight |
|----------------------------|--------------------|
| 5 Linseed oil              | 15 to 40           |
| 5 Triglyceryl-isolinoleate | 85 to 60           |

Example 2

|                           |          |
|---------------------------|----------|
| Linseed oil               | 15 to 40 |
| Triglyceryl-isolinolenate | 85 to 60 |

Example 3

|                          |          |
|--------------------------|----------|
| Perilla oil              | 15 to 40 |
| Triglyceryl-isolinoleate | 85 to 60 |

Example 4

|                           |          |
|---------------------------|----------|
| 15 Perilla oil            | 15 to 40 |
| Triglyceryl-isolinolenate | 85 to 60 |

Example 5

|                          |          |
|--------------------------|----------|
| 20 Soya bean oil         | 10 to 30 |
| Triglyceryl-isolinoleate | 90 to 70 |

Example 6

|                           |          |
|---------------------------|----------|
| 25 Soya bean oil          | 10 to 30 |
| Triglyceryl-isolinolenate | 90 to 70 |

Example 7

|                          |          |
|--------------------------|----------|
| 25 China-wood oil        | 40 to 60 |
| Triglyceryl-isolinoleate | 60 to 40 |

Example 8

|                           |          |
|---------------------------|----------|
| 30 China-wood oil         | 40 to 60 |
| Triglyceryl-isolinolenate | 60 to 40 |

35 In the examples of paint and varnish vehicles given the drying and semi-drying oils may be used either in the raw state, refined or in blown condition as desired. Various mixtures of the different oils also may be utilized. Further use may be made of other oils, for example oticica, poppy seed oil, sunflower oil, as well as fish and marine mammal oils heretofore used in paint and varnish coating compositions.

40 The mixture of oil and glyceride is heated to incorporate the fatty acid glyceride to form a homogeneous composition. Heating the oil and glyceride mixture to a temperature of 350 to 450 degrees F. for one-half to one hour is sufficient to produce a satisfactory product.

45 Suitable driers or drier combinations may be incorporated in the modified oil vehicles if desired, such as the acetate, resinate or linoleate of cobalt, manganese or lead.

50 The glyceride modified oil vehicles illustrated in Examples 1 to 8 may be compounded with suitable resins, natural or synthetic; for example, kauri, congo, damar, pontianak, manila, elemi, mastic or synthetic resins such as "Cumar," ester gum, phenol formaldehyde resin, glycerol-phthalic acid resin particularly of the oil soluble type or mixtures of these. The coating compositions employing the glyceride modified oil vehicles may be either air dried or baked to produce a dry, smooth, flexible, water-resistant film.

55 60 A baking temperature range between 250 to 400 degrees F. for one-half to one and one-half hours may be employed.

65 For the production of similar coating compositions wherein the film readily dries to a wrinkle finish surface, modified oil vehicles comprising large percentages of fatty acid glycerides having 3 or more conjugated double bond molecular structure are employed.

|                                                    |           |
|----------------------------------------------------|-----------|
| 70 Typical examples of wrinkling oil vehicles are: | Example 9 |
| Linseed oil                                        | 5 to 25   |
| 75 Triglyceryl-elaeostearate                       | 95 to 75  |

## Example 10

|                      |          |
|----------------------|----------|
| Linseed oil          | 5 to 25  |
| Triglyceryl-lacanate | 95 to 75 |

## Example 11

|                                |          |
|--------------------------------|----------|
| Linseed oil                    | 20 to 40 |
| Triglyceryl-octodecatetraenate | 80 to 60 |

## Example 12

|                           |          |
|---------------------------|----------|
| Perilla oil               | 5 to 25  |
| Triglyceryl-elaeostearate | 95 to 75 |

## Example 13

|                      |          |
|----------------------|----------|
| Perilla oil          | 5 to 25  |
| Triglyceryl-licanate | 95 to 75 |

## Example 14

|                                |          |
|--------------------------------|----------|
| Perilla oil                    | 20 to 40 |
| Triglyceryl-octodecatetraenate | 80 to 60 |

## Example 15

|                           |          |
|---------------------------|----------|
| Soya bean oil             | 5 to 20  |
| Triglyceryl-elaeostearate | 95 to 80 |

## Example 16

|                      |          |
|----------------------|----------|
| Soya bean oil        | 5 to 20  |
| Triglyceryl-licanate | 95 to 80 |

## Example 17

|                                |          |
|--------------------------------|----------|
| Soya bean oil                  | 10 to 25 |
| Triglyceryl-octodecatetraenate | 90 to 75 |

In compounding the oil compositions of Examples 9 to 17, the fatty acid glycerides are thoroughly incorporated with the oils to provide a homogeneous drying oil vehicle in a similar manner to that described in Examples 1 to 8. It will be understood also that raw, refined or blown drying oil's may be used in preparing the wrinkling oils. In general when using blown or prepolymerized oils less amount of the glyceride constituent is required to produce a product which will dry in a given time.

The glycerides having triple or more conjugated double bonds may also be blended with tung oil or oiticica, which are wrinkling oils, to modify their wrinkling characteristics. In like manner the incorporation of natural or synthetic resins and driers may be made.

The compositions comprising the modified drying oil may be applied as a film by flowing or spraying and baked at temperatures of the order of 250 to 350 degrees F. for one to two hours to produce a wrinkle finish. Enamels require somewhat longer and higher temperatures of baking. For thinning the paint oil vehicles, petroleum naphtha, toluol, or mixtures of the two may be employed.

Further in utilizing the wrinkling oils of Example 9 to 17 the use of various natural or synthetic resins may be made to provide a resinous type coating composition. Various resins may be added to the composition in order to modify the properties comprising natural and synthetic resins such as heretofore mentioned. When it is desired to give added flexibility to the films, a suitable plasticizing agent such as castor oil, dibutyl phthalate or tricresyl-phosphate may be incorporated. The paint oil compositions herein illustrated can also be used in making enamels and similar pigmented compositions. To produce such compositions 5 to 25% of a suitable pigment is ground into the glyceride modified oil or resinous oil composition and the required amount of thinner such as petroleum naphtha and the like is added.

Clear varnish-like compositions may be applied

over various articles and baked either to a wrinkle finish or a smooth glossy surface depending upon whether the oils are those of Examples 1 to 8 or the wrinkling oils of Examples 9 to 17. Thin coatings may also be applied over materials such as paper, foil, parchment and the like to produce a light transmitting sheet applicable for making various articles such as window shades, drapes, lamp shades and the like. The coating compositions of this invention may also be applied over metal, wood, pottery, glass, paper, leather and the like, and baked or air dried to a flexible, tough film. Various ornamental effects of the wrinkle finishes can be produced by varying the percentage of poly-conjugated double bond glyceride constituent in the paint oil. Other modified results of the finish may be obtained by variations in the method of applying the compositions. Further one or more coats may be applied to an article and dried and thereafter cellulose lacquer or like composition disposed thereover.

It will be understood that I desire to comprehend within my invention such modifications as come within the scope of my invention as described and the appended claims.

It will be further understood that the term "non-wrinkling drying oil," as used in the claims, is intended to encompass drying oils and semi-drying oils of the type used in the examples hereinbefore set forth.

Having thus fully described my invention, what I claim as new and desire to secure by Letters Patent is:

35. A drying oil vehicle for coating compositions comprising a non-wrinkling drying oil having admixed therewith a triglyceride accelerator consisting of a high molecular weight unsaturated fatty acid triglyceride compound having conjugated double bond linkage of the formula  $(-\text{CH}=\text{CH}-)_x$ , wherein  $x$  is equal to 4.

36. A drying oil vehicle for coating compositions comprising a non-wrinkling drying oil and a drying accelerator incorporated therewith consisting of an unsaturated fatty acid glyceride compound having conjugated double bond linkage of the formula  $(-\text{CH}=\text{CH}-)_x$ , wherein  $x$  is equal to 4.

37. A coating composition comprising a non-wrinkling drying oil to which is added a wrinkle producing fatty acid glyceride comprising poly-conjugated double bond linkage in the molecular structure together with a metallic drier for producing a wrinkling composition, said double bond linkage being of the formula  $(-\text{CH}=\text{CH}-)_x$ , wherein  $x$  is equal to 4.

38. A coating composition adapted for use as a quick drying coating, comprising a non-wrinkling drying oil having incorporated therewith a sufficient amount of a siccative to produce a wrinkling composition on drying, said siccative consisting of a fatty acid glyceride of an acid having the conjugated double bond structural formula  $R_1-(\text{CH}=\text{CH})_xR_2\text{COOH}$ , wherein  $R_1$  is an alkyl radical,  $R_2$  is an alkylene radical and  $x$  is equal to 4.

39. A coating composition adapted for use as a quick drying coating, comprising a non-wrinkling oil having admixed therewith sufficient amount of a siccative to produce a wrinkling composition on drying, said siccative comprising resinous material and a fatty acid glyceride compound having the conjugated double bond structural formula  $R-(\text{CH}=\text{CH})_x\text{COOH}$ , wherein  $R$  is an alkyl radical and  $x$  is equal to 4.

FOLSOM E. DRUMMOND.